

Sept. 15, 1959

R. F. GIBSON ET AL  
LIGHTWEIGHT AGGREGATE FURNACE PATCH LINING  
AND PROCESS OF APPLYING  
Filed Nov. 28, 1955

2,903,778

FIG. 1



FIG. 3



FIG. 2

INVENTORS

A. F. OLD  
R. F. GIBSON

BY

*A. F. Old*

ATTORNEY

1

2,903,778

**LIGHTWEIGHT AGGREGATE FURNACE PATCH LINING AND PROCESS OF APPLYING**

Richard F. Gibson, Albemarle, N.C., and Albert Floyd Old, Bremo Bluff, Va., assignors to Southern Lightweight Aggregate Corporation, Richmond, Va.

Application November 28, 1955, Serial No. 549,484

2 Claims. (Cl. 25—155.5)

This invention relates to concretes and more particularly to a lightweight aggregate concrete mix especially adapted for filling or patching holes in furnace or kiln linings and to an improved process for accomplishing this and producing an improved concrete.

Kilns, particularly those of the rotary type, are frequently in continuous operation on a twenty four hour seven day week basis and are used for many purposes well known in the art, requiring the application of heat to substantially continuously flowing raw materials of various kinds.

These raw materials are usually rough in texture, and their movement, including tumbling, through the kiln in combination with the high temperatures used tends to erode the linings by mechanical abrasion, thermal stresses and chemical interaction.

Although the lining material is selected for its superiority in resisting such forces, nevertheless, portions of it fail as a result of the factors mentioned so that it becomes necessary from time to time to replace all or portions of the lining.

Heretofore, the repair of lining areas of limited size has usually necessitated shut down of the kiln for a sufficient length of time for it to cool in order that workmen might enter and replace the lining which has been lost or needs repair. Since kilns are oftentimes of large size such as eight feet in diameter and over one hundred feet long and the linings are thick, and in view of the temperatures used (oftentimes exceeding 2000° F.) the time of shut down has been quite substantial. The substantial loss of productive output in addition to the fuel required to bring the kiln back to operating temperature has made the cost of such repairs large. A further factor is that because of the nature of the material available for patching or filling the voids, it has been necessary to apply these while the kiln is relatively cool and to permit them to cure or set up a substantial time prior to refiring of the kiln.

Accordingly, it is an object of the present invention to provide an improved concrete material having high abrasion resistance and low thermal conductivity characteristics.

A further object is to provide material which may be applied to fill in voids in kiln linings without waiting for the kiln to cool and which possesses superior characteristics.

A further object is to provide an improved method for patching or filling voids in kiln linings through the use of the improved material of the present invention.

These and other objects of the present invention will become apparent from the following description in conjunction with the accompanying drawing in which—

Fig. 1 is a fragmentary perspective of an end of a kiln with a hole in its lining and with a patch applied according to the present invention (a portion being removed for clarity of presentation),

2

Fig. 2, an enlarged section through the material of a patch; and

Fig. 3, a perspective, to an enlarged scale, of a portion of the surface of a part of the kiln wall illustrating the method of installing cleats from the exterior of the kiln.

Various materials have been used for kiln linings, both in monolithic and block or brick form. Among the desirable characteristics which lining materials should possess are those of high resistance to mechanical abrasion and low thermal conductivity. Lining materials vary rather widely in these characteristics.

Conventional lining materials heretofore known such as brick or ordinary concrete must be applied and permitted to cure without being subjected to thermal shock.

For example, the application of excessive heat to concrete formed from materials such as quartz sand and gravel causes concrete to disintegrate.

According to the present invention, lightweight aggregate having particular characteristics may be used together with certain cements such as Portland, slag or natural, and applied to the area of the kiln requiring patching without waiting for the kiln to cool. The resulting material is at least equal to and superior to many kiln lining materials with respect to abrasion resistance

and thermal conductivity. Furthermore the material of the patch usually stays in place longer than ordinary kiln brick; it has been found upon examination of the patching material after shutdown of the kiln for the replacement of the lining that such material has maintained

a hard smooth surface and is more firmly adhered to the kiln wall than the surrounding lining.

In producing the patching material, the lightweight aggregates referred to in our Patent 2,721,069 have been found to be especially efficacious. The aggregates there described are adapted for load bearing concretes and are produced from slates. For use in the present invention, these are graded by sieve analysis as described hereafter. One of these aggregates results from the expansion of a weathered argillaceous slate which has lain close to the surface of the earth for a substantial period of years and during this time has been subjected to repeated cycles of freezing and thawing, to erosion, and has been permeated to some degree with substances such as clay or silt that has flowed down into the voids. The result has been that the cleavage lines or planes have been broken or displaced. As a result when such material is graded to the desired size for heat treatment the individual particles are substantially free of cleavage lines.

The other aggregate described results from the heat treatment of certain non-argillaceous slate deposits in which the laminations occur at wide intervals such as 37" apart; as a result the crushed raw material is substantially entirely free of laminations.

The lightweight aggregate used as the aggregate in the material of the present invention is obtained as a result of the kiln heat treatment described in Patent 2,721,069. Following such kiln heat treatment, the aggregate is crushed and for the purposes of the present invention is sized or graded according to the following sieve analysis based on the American Society of Testing Materials specification:

| Sieve size or number: | Percentage by weight passing |
|-----------------------|------------------------------|
| 3/8"                  | 100                          |
| No. 4                 | 85 to 100                    |
| No. 16                | 40 to 80                     |
| No. 50                | 10 to 35                     |
| No. 100               | 5 to 25                      |

Test batches of concrete are made using Portland cement or equivalent (such as natural or slag cement) and

water, the cement factor running from approximately 5 to 7 bags (standard 94 lb.) per cubic yard of concrete. The water is held to a minimum, just sufficient to make the mix plastic enough to hand trowel, the water/cement ratio usually ranging from 3 to 1 up to 5 to 1 gallons per sack.

When an eroded area or void is found in the kiln, it is only necessary to stop operation of the kiln sufficiently long to apply the patch to the area. The kiln is rotated to bring the area on to the lower side preferably so that the mix may flow by gravity into the void. If the area is beyond reach from the end of the kiln by ordinary means, a pipe or the like may be used to convey the material to the area. Because of the heat present, the cement hardens almost immediately, the result being that operation of the kiln may be resumed as soon as the material is in place.

The abrasive resistance of the patching material is higher than that of brick ordinarily used and stays in place 3 to 5 times longer than ordinary brick. Similarly the "K factor" is lower than that of such brick and runs between 3.5-4.0 B.t.u. per hour per square foot per inch of thickness.

The foregoing method of patching is suitable for relatively small areas up to approximately 3 to 4 square feet. For larger areas it is preferable to weld cleats or rods or similar type projections to the interior of the shell to assist in retaining the patching material in place. If time and conditions permit, the projections may be attached by welding from the interior. This procedure, however, requires that the temperature be sufficiently low for a workman to work within the kiln.

In order to avoid the delay required for cooling of the kiln, the following described method may be used. Referring more particularly to Fig. 1, a kiln 10 is illustrated having a lining 11 of blocks or brick 12 adjacent to the end 13. In the end portion, there is a void 14 with patching material 15, shown in place at the rear portion thereof for illustrative purposes. Cleats 16 are welded to the shell 17 of the kiln and project inwardly. The illustrated cleats are angle iron welded in the designated place by cutting openings 18 with a torch or the like through which the cleats may project into the interior of the kiln, the openings being cut from the outside. After cutting of the openings the cleats are inserted therethrough and the end portions 19 joined by a weld 20 to the shell. As soon as the desired number of cleats are positioned, the batch of material may be poured into the location and operation of the kiln resumed.

It will be understood that cleats may be installed as described at a location in the kiln remote from its ends, and without requiring a workman to enter the kiln or be exposed to the temperatures therewithin. Of course, such cleats may be installed from within if the furnace is shut down. The concrete mix may be applied to the area by conventional means such as long-handled shovels, pipes, and the like.

Although the invention has been described in connection with the use of expanded lightweight aggregates produced from argillaceous and non-argillaceous slates, it is

believed that expanded lightweight aggregates produced from shales and clays may also be used.

Accordingly it will be understood that an improved concrete mix has been provided which may be poured onto a hot surface such as in a kiln, although its use is not so limited, and which withstands such heat without the necessity of slow curing, as with conventional mixes. The material provides a hard abrasion resistant patch, having low thermal conductivity and a high degree of adherence to the wall of the kiln.

Although particular applications have been described, it will be understood by those skilled in the art that the invention is not thus limited, but that equivalent materials and applications are within the scope of the invention and, therefore, the invention is only limited as defined in the following claims.

What is claimed is:

1. The method of filling a void in kiln lining resulting from the removal of the lining by erosion, cracking, and the like, comprising preparing a concrete mix using approximately 5½ to 7 bags of cement per cubic yard of concrete mix together with lightweight aggregate prepared from expanded particles of slate, the water/cement ratio being in the range of approximately 3 to 1 to 5 to 1, preparing the area of the void for the mix comprising cutting a plurality of openings from the exterior of the kiln wall through the kiln wall, such openings corresponding to the profile of projecting members, inserting a projecting member through each opening and retaining the tip of the projecting member in contiguous relation to the opening by the application of a weld between such end and the portion of the wall defining the opening, and pouring the mix into the void while the kiln is hot.
2. The method of filling a void in kiln lining resulting from the removal of the lining by erosion, cracking, and the like, comprising preparing a concrete mix, preparing the area of the void for the mix comprising cutting a plurality of openings from the exterior of the kiln wall through the kiln wall, such openings corresponding to the profile of projecting members, inserting a projecting member from said exterior through each opening and retaining the tip of the projecting member in contiguous relation to the opening by the application of a weld from said exterior between such end and the portion of the wall defining the opening, and pouring the mix into the void in contact with the portions of the projecting members extending thereto.

#### References Cited in the file of this patent

#### UNITED STATES PATENTS

|           |                |                |
|-----------|----------------|----------------|
| 1,091,567 | Eldred         | Mar. 31, 1914  |
| 1,316,298 | Gold           | Sept. 16, 1919 |
| 1,916,157 | Chappell       | June 27, 1933  |
| 2,124,865 | Winkler et al. | July 26, 1938  |
| 2,358,652 | Nicholas       | Sept. 19, 1944 |
| 2,504,185 | Debenham       | Apr. 18, 1950  |
| 2,564,009 | Hyche          | Aug. 14, 1951  |
| 2,607,700 | Vail           | Aug. 19, 1952  |
| 2,635,865 | Brumbaugh      | Apr. 21, 1953  |